

# UNITED STATES PATENT OFFICE.

WILLIAM FELDENHEIMER, OF LONDON, ENGLAND.

## SOAPLIKE DETERGENT AND THE MANUFACTURE THEREOF.

1,254,588.

Specification of Letters Patent. Patented Jan. 22, 1918.

No Drawing.

Application filed April 12, 1917. Serial No. 161,606.

*To all whom it may concern:*

Be it known that I, WILLIAM FELDENHEIMER, a subject of the King of England, residing at London, in England, have invented certain new and useful Improvements in Soaplike Detergents and the Manufacture Thereof, of which the following is a specification.

This invention is for improvements in or relating to soap-like detergents and the manufacture thereof by the boiling process with separation of glycerin, and has for its object to produce a good quality soap-like substance or "soap-stock" (that is the same substance when in the condition in which a true soap is known as soap-stock) from the lyes which have been separated from the soap-mixture during the ordinary process of manufacture and contain the glycerin as usual.

According to this invention, the separated lyes (or the mixture of lyes and curds which latter consists of particles of soap contained in the lyes) has added to it when at a temperature of between 80° to 90° C., ground maize-cones in the proportion of approximately 15% by weight of the lyes or the lyes estimated to be contained in the mixture.

Preferably after adding the ground maize-cones the temperature of the mixture is raised to boiling-point and when cooled it sets to a jelly which is found to possess all the properties of a good water-soluble soap.

Maize-cones are a form of finely ground maize well known in England, the maize being ground into hygroscopic cones so that the ground material feels granular.

If desired, about 15% by weight of china-clay can be added in addition to the ground maize-cones, while the lyes or soap-mixture is at 80° to 90° C., and when this is done, the mixture when cooled has the consistency of a thick white cream and still possesses many of the useful properties found in what is popularly known as a good water-soluble soap.

What I claim as my invention and desire to secure by Letters Patent is:—

1. The process of manufacturing a soap-like detergent or "soap-stock" from lyes such as commonly result from the boiling process with separation of glycerin in the manufacture of soap, consisting in adding to the lyes when at a temperature of between 80° to 90° C. with the glycerin therein, ground maize-

cones in the proportion of approximately 15% by weight of the lyes, substantially as set forth.

2. The process of manufacturing a soap-like detergent or "soap-stock" from lyes such as commonly result from the boiling process with separation of glycerin in the manufacture of soap, consisting in adding to the lyes containing the usual "curds," that is, soap particles, as well as the glycerin, when at a temperature of between 80° to 90° C., ground maize-cones in the proportion of approximately 15% by weight of the lyes estimated to be contained in the mixture, substantially as set forth. 70

3. The process of manufacturing a soap-like detergent or "soap-stock" from lyes such as commonly result from the boiling process with separation of glycerin in the manufacture of soap, consisting in adding to the lyes when at a temperature of between 80° to 90° C. with the glycerin therein, ground maize-cones in the proportion of approximately 15% by weight of the lyes, and finally raising the mixture containing the maize-cones 75 to boiling point before it is allowed to cool, substantially as set forth.

4. The process of manufacturing a soap-like detergent or "soap-stock" from lyes such as commonly result from the boiling process with separation of glycerin in the manufacture of soap, consisting in adding to the lyes when at a temperature of between 80° and 90° C. with the glycerin therein, ground maize-cones in the proportion of approximately 15% by weight of the lyes and 15% by weight of china-clay, substantially as set forth. 90

5. The process of manufacturing a soap-like detergent from the lyes containing glycerin resulting from soap manufacture, which consists in adding ground maize-cones to the lyes, substantially as set forth. 95

6. The process of manufacturing a soap-like detergent from the lyes containing glycerin resulting from soap manufacture, which consists in adding ground maize-cones to the lyes heated, substantially as set forth. 100

In testimony whereof I have signed my name to this specification in the presence of two subscribing witnesses.

WILLIAM FELDENHEIMER.

Witnesses:

A. M. HAYWARD,  
HAROLD H. SIMMONS.